

## UNITED STATES PATENT OFFICE

2,070,584

## PRODUCTION AND TREATMENT OF ARTIFICIAL FILAMENTS, THREADS, RIBBONS, AND THE LIKE

Henry Dreyfus, London, England

No Drawing. Application May 25, 1933, Serial No. 672,805. In Great Britain June 14, 1932

12 Claims.

(Cl. 8—20)

- This invention relates to the production and treatment of artificial filaments, threads, yarns, ribbons, foils and the like made of or containing organic derivatives of cellulose, and particularly to processes whereby materials having an increased extension and tensile strength may be obtained. This application is a continuation-in-part of application S. No. 378,684 filed July 16, 1929.
- U. S. Patent No. 1,709,470 describes processes in which cellulose acetate filaments are stretched beyond their elastic limit at any suitable stage of their manufacture, after the artificial silk is in the fully set and finished condition, the stretching being assisted, if desired, by means of "assisting agents" which swell the cellulose acetate materials, for example acetone, ethyl alcohol, formaldehyde or glycerine. Again, U. S. application S. No. 378,684 filed July 16, 1929 describes the stretching of filaments, threads and similar products containing cellulose acetate or other organic esters of cellulose while they are travelling from one point to another, the stretching being facilitated by the action of solvents or swelling agents for the cellulose derivative, and U. S. application S. No. 403,140 filed October 28, 1929, describes the advantages obtained by employing solvents in relatively high concentration to assist the stretch.
- U. S. application S. No. 573,424 filed November 6, 1931, describes a process for improving the properties of filaments, threads, yarns, ribbons and the like containing cellulose esters or ethers, and particularly their tensile strength, in which the materials are softened and then subjected to at least two stages of stretching, the tension being substantially removed between at least two of the stages, while retaining the plasticity or softness of the products.
- All these processes result in the production of filaments and other materials having increased tensile strength, but on the other hand such materials may have a relatively low extension. A method of obtaining materials which have both good tensile strength and also a satisfactory extension is described in U. S. application S. No. 611,240 filed May 13, 1932, according to which artificial filaments, yarns, ribbons and the like made of or containing organic derivatives of cellulose, and particularly wet spun products or dry spun products which have been submitted to a stretching operation, are treated with shrinking agents.

These specifications, therefore, relate either to processes for improving the tensile strength of

artificial filaments and other materials containing organic derivatives of cellulose by stretching them, or to improving the extension of artificial filaments and the like by a shrinking operation.

I have now discovered that the properties of artificial filaments, threads, yarns, ribbons, foils and the like made of or containing organic derivatives of cellulose, and particularly their extensibility and tensile strength, may be improved by treating them with shrinking agents in the absence of tension sufficient to stretch them and then subjecting them to a stretching operation. Preferably treatment with the shrinking agents is carried out so that the filaments and the like are not subjected to any tension, or at least only a moderate tension, but if a relatively high tension is applied, the tension should be subsequently decreased or removed, so that shrinkage or further shrinkage is possible.

The invention is especially of value in relation to the treatment of artificial materials made of or containing cellulose acetate and it will therefore be described with particular reference thereto. Its application, however, is by no means limited to such materials and it is also of value in connection with the treatment of materials containing other organic esters or mixed esters of cellulose, for example cellulose formate, propionate, butyrate and nitroacetate, methyl, ethyl, propyl, butyl and benzyl cellulose and other cellulose ethers or mixed ethers, and mixed cellulose ether-esters, for example, ethyl cellulose acetate and oxyethyl cellulose acetate.

The process of the present invention may be carried out as a separate operation distinct from the production of the materials, as, for example, in a bobbin to bobbin treatment or with skeins, hanks or other packages, or it may be applied continuously with the production of the artificial materials by wet or dry processes.

When the invention is applied to the treatment of artificial filaments, yarns and the like in hank form, the apparatus described in U. S. application S. No. 573,424 in connection with the application of stretch to such materials, or a modification thereof, may very conveniently be employed. This apparatus consists of a relatively long bath which, for the purposes of the present invention, will contain the shrinking agent, and which may be lined with a suitable material which is resistant to the action of such agent. A long screw fitted with a hand wheel or other suitable drive is arranged longitudinally along the top of the bath in which two rollers carried on suitable supports are posi-

tioned. One of the rollers is connected to the screw so that its position in the bath may be adjusted by rotating the screw, while the other is arranged so that it may be either fixed in one position or allowed to move freely along the bath. By means of the screw the distance of the roller carried on the screw from the other roller may be adjusted so as to stretch the hanks which are passed over the rollers. In applying this apparatus for the purpose of the present invention, any suitable means may of course be employed whereby the hanks are allowed to shrink by the desired amount. For example, hanks may be placed on the rollers and their distance apart adjusted so that the hanks are able to shrink to a certain definite and predetermined extent under the influence of the shrinking agent contained in the bath, or alternatively the roller which is not carried on the screw may be free to move longitudinally along the bath, so that the hanks can shrink freely, the shrinking of the yarn itself drawing the rollers nearer together. When sufficient shrinkage has taken place, stretching may be carried out in the same apparatus, as is described in U. S. application S. No. 573,424 referred to above. Thus the position of the "free" roller may be fixed, and the hanks stretched by rotating the screw, and thus causing the roller carried thereon to move away from the "free" roller. The agent used to bring about the shrinking may be the same as that employed for the softening process, or, if desired, it may be different, in which case, on completion of shrinking, the shrinking agent is removed and the bath then filled with the softening agent which it is desired to employ. Alternatively of course the stretching process may be carried out in any other suitable manner, for example as described in U. S. Patent No. 1,709,470.

Other methods by which shrinking may be carried out upon the materials in package form include the use of resilient bobbins, swifts or supports and of loosely wound packages, and in this connection, as well as in connection with the shrinking of materials during their travel from one point to another, referred to in greater detail below, reference is made broadly to the methods described in U. S. application S. No. 611,240.

Alternatively the shrinking operation may be carried out upon the artificial materials during the course of their travel from one point to another, as for example in a bobbin to bobbin winding operation or in the course of their production by dry or wet spinning processes. Thus, artificial filaments proceeding from a bobbin or other suitable package or from a dry or wet spinning apparatus may be passed around a positively driven roller, through a suitable shrinking bath and then wound on a second roller positively driven at a peripheral speed less than that of the first roller, so that the desired shrinking can take place. Alternatively nip rollers may be employed and/or the shrinking bath may itself be caused to flow in a direction counter to that of the travel of the artificial filaments or other materials so as to assist shrinkage. The use of liquid baths in motion for the purpose of restricting the tension applied to the artificial filaments is described in U. S. application S. No. 593,859 filed February 18, 1932, and the principles described therein may be applied to the present invention.

While the shrinking agents to be employed according to the present invention are preferably

applied by passing the materials through baths containing the agents, yet the invention is not limited to such methods. For instance, the shrinking agents may be applied in the vapour state by means of sprays and the like, or the materials may be caused to contact with rollers, pads, wicks or similar devices which are saturated with the shrinking agents. Again, low boiling liquids may be applied in the vapour state, or air or other gases saturated with the vapour of the shrinking agent may be passed over the artificial materials, and in this case the motion of the gases may be employed to assist the shrinking, using, for example, the principles disclosed in U. S. application S. No. 590,828 filed February 4, 1932.

Not only may the shrinking operation be carried out continuously with the production of the artificial materials by passing them from the coagulating bath or evaporative medium into a suitable shrinking bath, but, if desired, shrinkage may also take place simultaneously or substantially simultaneously, with the formation of the materials. For example, in the case of wet spinning, a positively driven guide roller or nip rollers may be suitably positioned in the coagulating bath and rotated at a peripheral speed less than that at which the artificial filaments and the like are extruded from the spinning orifices and thus by the use of suitable coagulating baths shrinkage may take place in the bath itself. If desired, a draw roller rotating at a peripheral speed substantially equal to that of extrusion may be positioned between the jets and the above mentioned guide or nip rollers. Suitable baths for this purpose are those containing solvents or latent solvents for the cellulose derivative as described in U. S. Patents Nos. 1,465,994 and 1,467,493, and U. S. applications S. Nos. 402,785 filed October 26, 1929, and 437,423 filed March 20, 1930, or coagulating baths containing the shrinking agents and/or diluents mentioned below may be employed.

In the case of dry-spinning, the evaporative atmosphere remote from the spinning jets may contain a shrinking agent, so that the artificial materials are first substantially coagulated and are then shrunk. A positively driven roller or rollers having a peripheral velocity less than that of the speed of extrusion may be arranged in a suitable position either inside or outside the cell, and if desired an intermediate roller, as described above in relation to wet-spinning, may also be employed. An outlet for the atmosphere containing shrinking agent and an inlet for the main evaporative atmosphere may be provided at points between the inlet for shrinking agent, which will be remote from the jets and the outlet for the main evaporative atmosphere in the vicinity of the jets.

Amongst suitable shrinking agents for use in accordance with the present invention may be mentioned acetic acid, formic acid, lactic acid, diacetone alcohol, acetone, aliphatic alcohols, e. g. ethyl alcohol, mono-and di-ethers or esters or ether-esters of olefine or polyolefine glycols, for example mono- and di-ethyl ethers of ethylene glycol, glycol mono-acetate, methyl glycol mono-acetate, dioxane and other cyclic ethers, for example methylene ethylene oxide, the mono methyl and ethyl ethers of propylene glycol and the mono ethyl ethers of diethylene glycol, phenols, mono, di- and tri-acetins, dichlorethylene, ethyl lactate, diethyl tartrate and other substances or solutions or mixtures having swelling, solvent or latent solvent action upon the cellu-

lose derivative. Such agents may, if desired, be used in aqueous solution or in admixture with organic diluents.

Particularly suitable for the purpose of the present invention are agents which, at least at ordinary temperatures, are not solvents for the cellulose derivative, but which are capable of swelling it to a high degree. Examples of such agents are methylene chloride, ethylene chloride, ethyl acetate, chloroform and tetrachlorethane. These agents, for example, methylene chloride, chloroform and dichlorethylene, when mixed with comparatively small proportions of an alcohol or certain other liquids, become capable of dissolving cellulose acetates, and they are usually referred to as latent solvents for cellulose derivatives. Such latent solvents are particularly advantageous for use in accordance with the present invention, but they are preferably not employed in admixture with alcohols or other agents which are capable of converting them into true solvents, but either alone or in admixture with diluents or substances having little or no solvent or swelling action at ordinary temperatures. In the event of their being used in conjunction with alcohols or similar acting substances, proportions should be chosen so that a true solvent mixture is not formed.

As suitable diluents for use in connection with the present invention may be mentioned water, glycerol, glycol or other hydroxy compounds, though preferably water-immiscible liquids are employed. Examples of such liquids are benzene, toluene and other cyclic hydrocarbons, benzene, kerosene, carbon-tetrachloride, petrol ether, trichlorethylene, perchlorethylene and other chlorinated or halogenated compounds which are inert or relatively inert towards the cellulose derivative. High boiling diluents, for example tetrahydro-naphthalene and decahydronaphthalene, may also be employed.

As is described in U. S. application S. No. 611,240, very considerable shrinkages may be produced in the absence of tension by treatment of artificial materials with pure methylene chloride, chloroform, tetrachlorethane or similar latent solvents, and since, according to the present invention, the materials are to be subsequently stretched, a higher degree of shrinkage is in general found desirable than when shrinking follows stretching as in the process of the above specification. Thus, the shrinkage produced according to the present invention may be of the order 15 to 25 or 35%, or even more. Any desired restriction of the shrinkage may be effected by controlling the concentration of the shrinking agent, the time of treatment and/or by carrying out the process under sufficient tension to prevent more than the desired shrinkage. Thus when using a mixture of methylene chloride and benzene in a proportion of 50:50 by volume, with artificial materials obtained from commercial acetone-soluble cellulose acetate, the process may be carried out so that a shrinkage of 25-30% is effected.

Stretching of the materials after shrinking may be carried out either immediately or after a lapse of time. Preferably however the stretching process is combined with the shrinking process, the whole forming a continuous operation.

According to the present invention, the agent employed in effecting shrinkage may be relied upon to soften the materials sufficiently for stretching, or the materials may be treated with further quantities of the same or a different agent. Alternatively, the agent employed for producing

shrinkage may be partially or completely removed, the materials being then treated with a softening agent, which in this case also may be the same as or different from that employed to effect shrinkage, and stretched.

Thus hanks which have been shrunk in the apparatus described above may be stretched without removing them from the rollers by increasing the distance apart of the said rollers.

Again, artificial filaments which have been subjected to a shrinking operation in the course of their travel from one point to another may be carried from the shrinking bath into another bath in which they are stretched, either in a single stage, as is described in U. S. application S. No. 378,684, or in two or more stages, as described in U. S. application S. No. 573,424. Moreover the shrinking and stretching may take place in the same bath, e. g. by passing the filaments or threads first round a roller rotating at a suitable speed either before or upon their entrance into the bath, then round another rotating at a smaller peripheral speed to allow of shrinkage, and then round one or more rotating at increasingly higher speeds in order to produce the desired stretch. If desired, a "rest" period may be arranged by rotating two or more successive rollers at the same peripheral speed so that during this portion of their travel the filaments undergo neither shrinkage nor extension. Further, particularly when filaments or yarns which have been shrunk in a previous operation are being stretched, means for restricting the action of the stretching force in the softening bath may be employed, as described for example in my co-pending U. S. application S. No. 672,800 filed on even date herewith.

Prior to stretching the materials may be subjected to two or more softening treatments with softening agents of different strengths, as described in U. S. application S. No. 638,776 filed October 20, 1932.

Again, filaments and the like which have been subjected to a shrinking operation may issue from the bath in a sufficiently softened state to be subjected to the stretching operation without further treatment, particularly if relatively non-volatile shrinking agents are employed, or they may be maintained in or brought to a sufficiently plastic condition merely by spraying, contact with wicks or rollers impregnated with the softening agent, or in any suitable manner.

The agents employed to promote shrinkage or allow of stretching are preferably removed on the completion of the operation, for example by evaporation in the case of relatively volatile agents or by a suitable bath treatment. Removal of the agent or agents may be carried out in a single operation on completion of the stretching process, e. g. by washing with solutions of the softening agent in successively decreasing concentrations, or the shrinking agent may, if desired, be removed before stretching takes place. In general, it will be necessary in such cases to assist stretching by treatment of the materials with softening agents. If desired, the softening bath or a portion thereof may be diluted and employed for washing the materials, as described in U. S. application S. No. 668,071 filed April 26, 1933.

The process of the present invention may, as described above, be carried out upon individual filaments, threads, or yarns, either in the form of hanks or other packages or during their travel from one point to another. It may further, if desired, be applied to a warp of threads from a suitable creel or beam, the warp being carried,

e. g. between nip rollers or draw rollers suitably driven so as to allow of a shrinkage.

Thus a warp of threads may be carried by means of draw rollers through a shrinking bath, the peripheral speeds of the rollers being suitably adjusted to allow of the desired shrinkage, and then in contact with further rollers, either in the same bath or forming part of a separate piece of apparatus, for the purpose of stretching them. If desired, one or more intermediate rollers may be employed in order to allow of a rest period between shrinking and stretching.

The process may also be applied, if desired, to mixed yarns and the like, for example, yarns containing filaments or threads of an organic derivative of cellulose together with filaments or threads of natural textile materials, for example, cotton, wool, pure silk and the like, and special effects may thus be obtained.

Various methods of carrying out the invention have been described above, but it is of course evident that the invention is by no means limited thereto, but comprises broadly the treatment of artificial filaments, threads, yarns, ribbons and the like containing organic derivatives of cellulose with shrinking agents, so as to bring about shrinkage, combined with a subsequent stretching process, in order to obtain products having an improved extensibility and tensile strength.

The following examples illustrate methods of carrying out the invention but it must be clearly understood that they are not to be considered as limiting it in any way.

#### Example 1

A number of cellulose acetate threads proceeding from a creel of bobbins in parallel formation are carried under a roller and through a reed submerged in the shrinking agent contained in a relatively long bath (of the order of 100 feet). This roller rotates at a peripheral speed of 7-8 metres per minute. About 20 feet from the first roller the threads contact with a second roller rotating at a lower peripheral speed so that a shrinkage of the order 15-20% may take place. From this roller the threads pass through a reed to a third roller rotating at a peripheral speed of 15-20 metres per minute, and thence out of the bath to washing, drying and winding devices. The agent used in the bath for both the shrinking and stretching stages is a solution consisting of 65% methylene chloride and 35% benzene.

#### Example 2

Cellulose acetate yarn in cake form is immersed in a shrinking agent consisting of 80% ethyl acetate and 20% toluene for a period of 5-10 minutes. The cake is then removed and the shrinking agent is then driven off, e. g. by means of a current of warm air. The thread is then led from the cake (which is carried on a suitable support) to a feed roller which is fixed in a bath and which rotates at a peripheral speed of 5-6 metres per minute. The roller is immersed in a softening agent consisting of a 45-50% aqueous solution of dioxane. From the first roller the threads pass to a second roller rotating at a peripheral speed of 20-25 metres per minute so that a stretch of about 400% is obtained. The threads then pass from the bath to washing, drying and winding devices.

#### Example 3

A number of cellulose acetate threads are shrunk and stretched as in Example 1, except

that a 45-50% aqueous solution of dioxane is employed.

The materials obtained according to any of the above examples have an increased tensile strength and an improved extension.

What I claim and desire to secure by Letters Patent is:—

1. Process for the manufacture of artificial filaments, threads, yarns, ribbons, foils and like materials containing organic derivatives of cellulose, which comprises treating the materials with shrinking agents under such conditions that shrinkage occurs to the extent of at least 15% of the original length and subsequently stretching the materials beyond their original length to increase their tenacity.

2. Process for the manufacture of artificial filaments, threads, yarns, ribbons, foils and like materials containing cellulose acetate, which comprises treating the materials with shrinking agents under such conditions that shrinkage occurs to the extent of at least 15% of the original length, and subsequently stretching the materials to a length at least of the order of 200% of their original length to increase their tenacity.

3. Process for the manufacture of artificial filaments, threads, yarns, ribbons, foils and like materials containing organic derivatives of cellulose, which comprises treating the materials with shrinking agents under such conditions that shrinkage of the order of 20 to 25% occurs, and subsequently stretching the materials to a length at least of the order of 200% of their original length to increase their tenacity.

4. Process for the manufacture of artificial filaments, threads, yarns, ribbons, foils and like materials containing cellulose acetate, which comprises treating the materials during their travel from one point to another with shrinking agents under such conditions that shrinkage of the order of 20 to 25% occurs, and subsequently stretching the materials beyond their original length to increase their tenacity.

5. Process for the manufacture of artificial filaments, threads, yarns, ribbons, foils and like materials containing organic derivatives of cellulose, which comprises treating the materials with latent solvents for the organic derivatives of cellulose under such conditions that shrinkage occurs to the extent of at least 15% of the original length, and subsequently stretching the materials beyond their original length to increase their tenacity.

6. Process for the manufacture of artificial filaments, threads, yarns, ribbons, foils and like materials containing organic derivatives of cellulose, which comprises treating the materials with latent solvents under such conditions that shrinkage of the order of 20 to 25% occurs, and subsequently stretching the materials to a length at least of the order of 200% of their original length to increase their tenacity.

7. Process for the manufacture of artificial filaments, threads, yarns, ribbons, foils and like materials containing cellulose acetate, which comprises treating the materials with latent solvents selected from the group consisting of ethylene chloride, chloroform, tetrachlorethane and ethyl acetate, under such conditions that shrinkage of the order of 20 to 25% occurs, and subsequently stretching the materials beyond their original length to increase their tenacity.

8. Process for the manufacture of artificial filaments, threads, yarns, ribbons, foils and like

materials containing cellulose acetate, which comprises treating the materials with methylene chloride under such conditions that shrinkage of the order of 20 to 25% occurs, and subsequently stretching the materials to a length at least of the order of 200% of their original length to increase their tenacity.

9. Process for the manufacture of artificial threads, yarns, ribbons, foils and like materials containing cellulose acetate, which comprises as a continuous operation treating the materials with latent solvents selected from the group consisting of ethylene chloride, chloroform, tetrachlorethane and ethyl acetate, under such conditions that shrinkage of the order of 20 to 25% occurs, and subsequently stretching the materials beyond their original length to increase their tenacity.

10. Process for the manufacture of artificial threads, yarns, ribbons, foils and like materials containing cellulose acetate, which comprises as a continuous operation treating the materials with methylene chloride under such conditions that shrinkage of the order of 20 to 25% occurs,

and subsequently stretching the materials beyond their original length to increase their tenacity.

11. Process for the manufacture of artificial threads, yarns, ribbons, foils and like materials containing cellulose acetate, which comprises as a continuous operation treating the materials with methylene chloride under such conditions that shrinkage of the order of 20 to 25% occurs, and subsequently stretching the materials beyond their original length to increase their tenacity in the same treatment bath.

12. Process for the manufacture of artificial filaments, threads, yarns and like materials having a basis of cellulose acetate, which comprises as a continuous operation drawing the materials in warp formation through a bath containing a shrinking agent under such conditions that along part of their path through the bath the materials undergo shrinkage to the extent of 20 to 25% of their original length and then stretching the materials to a length greater than their original length along a further part of their path through the bath to increase their tenacity.

HENRY DREYFUS.